

# United States Patent

[19]

Van Stratum et al.

[11] 3,823,453

[45] July 16, 1974

[54] **METHOD OF MANUFACTURING AN INDIRECTLY HEATED CATHODE AND CATHODE MANUFACTURED ACCORDING TO THIS METHOD**

29/492, 25.15; 313/270, 337; 117/49; 219/92

[75] Inventors: **Antonius Johannes Alberta Van Stratum; Theodorus Hendrikus Weekers, both of Emmasingel, Eindhoven, Netherlands**

[56]

## References Cited

### UNITED STATES PATENTS

|           |         |                       |          |
|-----------|---------|-----------------------|----------|
| 1,897,933 | 2/1933  | Guthrie et al.....    | 117/49 X |
| 2,726,308 | 12/1955 | Cinamon.....          | 219/92 X |
| 2,970,204 | 1/1961  | Piceu et al.....      | 219/92   |
| 2,978,606 | 4/1961  | Kahl.....             | 313/270  |
| 3,535,757 | 10/1970 | Nestleroth et al..... | 29/25.14 |

[73] Assignee: **U.S. Philips Corporation, New York, N.Y.**

*Primary Examiner*—Roy Lake

[22] Filed: **Nov. 29, 1972**

*Assistant Examiner*—J. W. Davie

[21] Appl. No.: **310,347**

*Attorney, Agent, or Firm*—Frank R. Trifari

[30] **Foreign Application Priority Data**

Dec. 16, 1971 Netherlands ..... 7117226

[52] **U.S. Cl.** ..... **29/25.14, 29/484, 313/337**

[51] **Int. Cl.** ..... **H01j 9/00**

[58] **Field of Search** ..... **29/25.13, 25.14, 484, 488,**

[57]

## ABSTRACT

A cathode cap is welded to a metal cylinder over a black sintered metal layer which contains from 60 to 10 percent by weight of metal oxide and which covers the whole cylinder.

**4 Claims, 1 Drawing Figure**



PATENTED JUL 16 1974

3,823,453



**METHOD OF MANUFACTURING AN INDIRECTLY HEATED CATHODE AND CATHODE MANUFACTURED ACCORDING TO THIS METHOD**

The invention relates to a method of manufacturing an indirectly heated cathode in which a nickel cap as a support of the emissive material is welded to one end of a metal cylinder which is coated with a black layer. The invention furthermore relates to a cathode obtained according to said method.

It is known that a short heating time can be obtained in an indirectly heated cathode consisting of a nickel cap which supports the emitting material and which is welded to a metal cylinder, if the inner surface and the outer surface of the cylinder are coated with a black layer. The black layer on the inside rapidly absorbs thermal energy from the filament, while the black outside radiates much thermal energy at high temperature so that a comparatively large heating energy is required to keep the cathode at the emission temperature. This high thermal energy ensures a short heating time. The black layer can be obtained in a simple manner by oxidizing the material of the cylinder which usually consists of nickel or of a nickel-chromium alloy, before the cap is provided.

The drawback, however, is that the end to which the nickel cap is to be welded must first be cleaned since welding of the cap to the oxide layer is not readily possible. This cleaning, however, is time-consuming.

The oxidation after the cap has been welded to the cylinder is disadvantageous since the cap also oxidizes as a result of which the reducers which are present in the nickel of the cap are converted into oxides, which produces emission difficulties.

The drawbacks of the said methods can be avoided if, according to the invention, the cylinder is previously coated with a layer of a suspension comprising one or more suitable refractory metals and one or more metal oxides in powder form, after which the layer is dried and sintered in a reducing atmosphere, the nickel cap is slid over one end of the cylinder coated with the sintered layer and is then welded to said end. Although the sintered layer generally still comprises metal oxide, it has been found that welding does not present any difficulties. A layer consisting of a mixture of tungsten and aluminium oxide has proved to be very suitable. A layer of molybdenum and aluminium oxide has also proved to be suitable. The quantity of tungsten in the suspension for the layer to be provided may be from 40 to 90 percent by weight, the quantity of aluminium oxide from 60 to 10 percent by weight. However, the suspension may also comprise tungsten or molybdenum and their oxides.

The invention will be described in greater detail with reference to an embodiment and a drawing the FIGURE of which is a cross-sectional view through a cathode obtained by means of the method according to the invention.

Reference numeral 1 in the FIGURE denotes a chromium-nickel cylinder (20 percent by weight Cr, 80

percent by weight Ni) which is coated with a sintered black layer 2 consisting of 60 percent by weight of tungsten and 40 percent by weight of aluminium oxide.

For that purpose, the surface of the cylinder 1 is dipped in a suspension containing, for example, 2 litres of methylisobutylketone in which 160 g of nitrocellulose have been dissolved and in which 720 g of tungsten powder and 480 g of  $Al_2O_3$  have been suspended. The layer is then dried and sintered in a hydrogen atmosphere at 1,200° C for 60 minutes. The aluminium oxide prevents the formation of an alloy between the tungsten and the nickel of the substratum which would decrease the radiation of the layer 2. A long cylindrical tube is preferably coated and after sintering cut into parts of the desired length. A nickel cap 3 is slid over one end of the coated cylinder 1, 2 and welded to the cylinder 1, 2, for example, by means of spot welds. The emissive layer 4 is provided on the cap 3. The cap comprises strips 5 with which the cathode can be connected.

Although in addition to tungsten the layer 2 comprises 40 percent by weight of  $Al_2O_3$  powder, it has been found that welding of the cap 3 does not present any difficulties. A heating member is afterwards provided in the cylinder 1. It has been found that the layer 2 maintains a constant black colour throughout the life of the cathode.

Although a single embodiment of a cathode has been described, cathodes which have been shaped in a different manner can also be manufactured by means of the method according to the invention. For example, the cap 3 may be provided with a flange for the connection in the electrode system.

What is claimed is:

1. A method of manufacturing an indirectly heated cathode, comprising the steps of providing a metal first body and a nickel cap member, coating said metal first body with a layer consisting essentially of at least one refractory metal and at least one metal oxide in powder form, sintering said coated first body in a reducing atmosphere to provide a black layer thereon, and then welding said nickel cap at one end of said coated first body, whereby said nickel cap provides a support for emissive material for said cathode.

2. A method as claimed in claim 1, wherein said first body is thus coated by dipping in a suspension which consists essentially of from 40 to 90 percent by weight of tungsten and from 60 to 10 percent by weight of aluminium oxide.

3. An indirectly heated cathode, comprising a metal first body coated with a sintered metal layer essentially consisting of from 60 to 10 percent by weight of metal oxide and the balance a metal, further comprising a cap welded to said first body over the sintered layer, and an emissive material provided on said cap.

4. An indirectly heated cathode as defined in claim 3, wherein said metal is at least one of molybdenum and tungsten and said metal oxide is at least one of aluminium oxide, molybdenum oxide, and tungsten oxide.

\* \* \* \* \*